

# UNITED STATES PATENT OFFICE.

WILLIAM M. KOON, OF TROY, NEW YORK.

## FIRE-KINDLING COMPOSITION.

SPECIFICATION forming part of Letters Patent No. 278,436, dated May 29, 1883.

Application filed March 23, 1883. (No specimens.)

*To all whom it may concern:*

Be it known that I, WILLIAM M. KOON, of the city of Troy, county of Rensselaer, and State of New York, have invented a new and useful Improvement in Fire-Kindling Compounds, of which the following is a specification.

My invention relates to a composition of combustible ingredients, the proportion in which the latter are used, and the manner in which they are mixed to produce a fire-kindling composition; and my invention consists, as will hereinafter be more fully described, in a combination of broken corncobs, sawdust, tan-bark, pitch, resin, kerosene-oil, and paraffine, mixed in the proportions and in the manner as subsequently described herein, the object of my improvement being to utilize these well-known combustibles in such a mixed proportion of each so as to produce a composition that will burn long enough and hot enough to ignite the coal in the stove when the kindling is placed beneath the latter, and which will be free from the objections made to the well-known combinations of material used for the same purpose.

It is a well-known fact that when the volatile compounds of hydrocarbon—such as kerosene or paraffine—or when pitch or resin are employed to saturate carbonaceous material for fire-kindling uses, unless mixed with slower-burning combustibles, they burn too rapidly, the more volatile elements being burned as evolved gases above the coal that they are intended to ignite, and if too large a proportion of pitch or resin is used the mass will adhere, which is objectionable. To obviate these difficulties and to produce a composition that will be free from adhesive tendencies, adapted to burn not too fast and still produce heat enough to ignite anthracite coal, in carrying out the purposes of my invention I use the following proportions of material: three bushels of coarsely broken-up corncobs, one peck of sawdust, one-half peck of tan-bark, six pounds of pitch, four pounds of resin, five quarts of kerosene-oil, and three pints of paraffine. To mix these materials the pitch and resin are melted together, and while warm the paraffine is added, and lastly the kerosene-oil. When this has

been done the previously-mixed carbonaceous material, consisting of the corncobs, tan-bark, and sawdust, is saturated with the liquid produced from the elements before described. The proportion of resin and pitch used then dry-coats the surfaces of the carbonaceous particles, so that they will not adhere, and as thus prepared the composition is put up in tin cans or packages to be sold as merchandise.

I am well aware that compositions of this class, broadly considered, are not new, and I am also aware that my invention, as an improvement thereon, is limited to the combination of materials used, the proportion in which each of them is used, in connection with the manner of uniting them and packing them.

I am well aware that corncobs saturated with kerosene-oil and other hydrocarbons have been used for a like purpose before; and I am also aware that wood-sawdust and spent tan-bark have been treated with paraffine or resin oil for the same use; hence, independently of my better method of using these elements, their combination with others which I employ, and the proportions of the materials used, I disclaim them.

It will be readily understood that the before-named older saturations of wood-sawdust and spent tan-bark with paraffine or resin oil, or corncobs with kerosene-oil, would be unstable, from the volatile character of all kinds of hydrocarbon liquid; but when such saturations are fixed by proper proportions of resin and pitch they are rendered permanent.

Having thus described my invention, what I claim, and desire to secure by Letters Patent, is—

A composition for fire-kindling, consisting of corncobs, sawdust, tan-bark, pitch, resin, kerosene-oil, and paraffine, when mixed together in the proportions named and in the manner set forth, to be packed for use as herein described.

Signed at Troy, N. Y., this 21st day of March, 1883.

WILLIAM M. KOON.

Witnesses:

CHARLES S. BRINTNALL,  
STANLEY M. HOLDEN.